

F. W. THOMAS.  
PHONOGRAPH DISK RECORD.  
APPLICATION FILED JULY 28, 1914.

1,134,774.

Patented Apr. 6, 1915.

Fig. 1



Fig. 2



Fig. 3



Fig. 4



Fig. 5



Fig. 6



WITNESSES

F. D. Sweet?

C. Broadway

INVENTOR

Frederic W. Thomas.

BY Munro Co.

ATTORNEYS

# UNITED STATES PATENT OFFICE.

FREDERIC W. THOMAS, OF NEW CITY, NEW YORK.

## PHONOGRAPH DISK RECORD.

1,134,774.

Specification of Letters Patent.

Patented Apr. 6, 1915.

Application filed July 28, 1914. Serial No. 853,607.

To all whom it may concern:

Be it known that I, FREDERIC W. THOMAS, a citizen of the United States, and a resident of New City, in the county of Rockland and State of New York, have invented a new and Improved Phonograph Disk Record, of which the following is a full, clear, and exact description.

This invention relates to phonograph disk records.

In disk records now in use and heretofore proposed there are certain inherent objections which it is the general object of the present invention to overcome by the production of a record which will give out mellow and pleasing sounds, do away with false, high notes, screechy and sharp noises, give a truer and more natural reproduction of sounds, and reproduce the human voice and other sounds more naturally. These results are unattained in the present disk records, owing to the fact that the disk body is of a hard, resonous nature. By the present invention the body of the record is permanently soft, yielding or cushiony, and hence non-sonorous, so that a more natural reproduction of sounds is possible without screechy noises or sharp notes.

In carrying out the invention the body of the record is made of a pad of felt, wood pulp or other fibrous material which is impregnated with a suitable material, such as asphalt or a composition in which the asphalt is the main constituent. This asphalt serves to impart permanent softness and non-resonance to the disk body, so that the record material applied to the surface thereof will be backed by a continuously soft cushion, whereby the objections to the present disk records are wholly overcome. A record of this type has the advantage of cheapness and simplicity of construction, indestructibility, stability sufficient to prevent cracking of the record material in the use and handling of the record, and superior tone qualities.

For a more complete understanding of the invention reference is to be had to the accompanying drawing taken in connection with the following description and appended claims.

In the accompanying drawing, which illustrates certain embodiments of the invention, and wherein similar characters of reference indicate corresponding parts in all the views, Figure 1 is a plan view of the improved disk record with a portion of the

record material broken away; Fig. 2 is an enlarged diametrical section; Fig. 3 is a plan view of a modified form of disk record; Fig. 4 is an enlarged diametrical section thereof; Fig. 5 is a plan view of a ring form of record; Fig. 6 is a diametrical section thereof.

Referring to the drawing, A designates a sound record of disk form which comprises a fibrous core or body 1 which has on one or both sides thereof the usual record material 2, so that in external appearance the record is like those in common use, except that at the center the fiber core or body 1 is exposed. This core may be made of wood pulp, felt or any other suitable material which has sufficient rigidity to support itself. The portion of the fibrous body 1 immediately under the record material 2 is in a permanently soft or non-resonant condition, due to the fact that it is impregnated with a suitable material, such as non-hardening asphalt or a composition in which asphalt or equivalent material is the principal ingredient. It is unnecessary to impregnate the central part of the disk where the record material does not appear, and this is brought out by the coarse and fine stippling, the coarsely stippled portion 3 being impregnated with the asphalt and the finely stippled portion 4 being unimpregnated. The fibrous material impregnated with asphalt and exposed for a long time to the action of the weather, retains its softness for an indefinite length of time, and consequently by inclosing the impregnated portion of the fibrous body with the practically non-porous record material, the fibrous body of the record will be practically of permanent softness or non-resonance.

In the record B shown in Figs. 3 and 4, the fibrous body 1<sup>b</sup> is rolled or pressed throughout that portion which is to receive the record material, and on this portion the record material 2<sup>b</sup> is applied after the fibers have been thoroughly impregnated with asphalt or the like. The record material is flush with the center of the fibrous body of the disk, making the latter of the same thickness throughout.

In the form of the invention shown in Figs. 1 to 4 inclusive there is a central aperture 5 to receive the post of the turntable of the phonograph, but the record may be made of annular form, as shown in Figs. 5 and 6. In this case the record C has an an-

nular body or core 6 of fibrous material that is impregnated throughout with asphalt or a compound thereof, and the record material 7 covers the upper and lower surfaces 5 and the inner and outer edges, thereby wholly incasing the core.

In making a record the softening material, which may be hot asphalt, asphalt with volatile oils, asphalt and twenty or twenty-10 five per cent. tar in hot condition, or asphalt and hot coal tar with volatile oils, is applied to the fibrous body or pad either by dipping the latter in the material or spreading the material on the opposite faces thereof until 15 the fibers are thoroughly impregnated. The pad is then dried, but in drying the pad remains soft, cushiony and non-sonorous. The record material is then applied to the impregnated part of the pad, and since this 20 material is hot when applied there will be a firm adhesion between the pad and record material, the asphalt also contributing to this result, so that there is no danger of the record material scaling or separating from 25 the pad.

From the foregoing description taken in connection with the accompanying drawing, the advantages of the construction and method of operation will be readily understood by those skilled in the art to which the 30 invention appertains, and while I have de-

scribed the principle of operation, together with the device which I now consider to be the best embodiment thereof, I desire to have it understood that the device shown is 35 merely illustrative and that such changes may be made when desired as are within the scope of the appended claims.

Having thus described my invention, I claim as new and desire to secure by Letters 40 Patent:

1. A sound record comprising a fibrous body, and a record material thereon, said body being impregnated with a non-hardening asphaltic material serving to render the body permanently non-sonorous and to cement the record material to the body.

2. A sound record comprising a fibrous body impregnated solely with asphalt, and record material applied to the impregnated body.

3. A sound record comprising a fibrous body impregnated with a non-hardening asphalt, and a surface layer of hard record material connected with said body.

In testimony whereof I have signed my name to this specification in the presence of two subscribing witnesses.

FREDERIC W. THOMAS.

Witnesses:

CHATTEN BRADWAY,  
GEORGE H. EMSLIE.